

Sept. 14, 1937.

E. C. DOMM

2,093,238

## PLATING OF WIRE

Filed Dec. 19, 1935



5 INVENTOR.  
ELGIN CARLETON DOMM

BY

McConkey & Booth

ATTORNEY'S.

## UNITED STATES PATENT OFFICE

2,093,238

## PLATING OF WIRE

Elgin Carleton Domm, Niles, Mich., assignor to  
 National Standard Company, Niles, Mich., a  
 corporation of Michigan

Application December 19, 1935, Serial No. 55,202

2 Claims. (Cl. 91—68.2)

This invention relates to the plating of wire, and is illustrated as carried out in plating a steel wire with zinc and then electrolytically depositing an outer coating of copper thereon.

5 In one desirable arrangement of the novel apparatus used, the wire (after suitable cleaning) is passed into a bath of molten zinc (or other metal to be plated thereon), where it remains long enough not only to receive a coating of zinc galvanized thereon but also to have its temperature raised to that of the zinc bath (e.g. about 840° F.). Preferably the wire, after leaving this bath is quenched, by passing over a wet roller or the like, to solidify and set the zinc coating without, however, substantially lowering the temperature of the wire.

As quickly as possible thereafter, and still at a temperature greatly in excess of the temperature of boiling water (e.g. at around 650° or 700° F.), passes directly into a hot aqueous electrolytic plating solution, preferably of copper cyanide. The hot plating solution is acted on by the wire at its still higher temperature, so that it has an immediate effect as soon as the wire enters the bath of cleaning the zinc surface and starting the 25 deposition of the copper on the zinc under the most favorable conditions, so that an extremely adherent coating is produced which, during storage after the plating is completed, is gradually absorbed by the zinc to form a thin coating of brass to which rubber can successfully and firmly be vulcanized.

The plating apparatus is of novel construction and arrangement designed to secure continuous effective circulation of fresh solution about the 35 wire being plated. This construction, and the novel composition of the solution and effective desirable current strength, and other novel and desirable features, will be apparent from the following description of the plating of a series of 40 wires in the novel apparatus illustrated in the accompanying drawing, in which:

Figure 1 is a top plan view of the apparatus;

Figure 2 is a section through the zinc plating tank, on the line 2—2 of Figure 1;

45 Figure 3 is a transverse section through the copper plating apparatus on the line 3—3 of Figure 1; and

Figure 4 is a longitudinal section through the copper plating apparatus, on the line 4—4 of 50 Figure 1.

In the apparatus illustrated, a series (e. g. ten) of steel wires 10 are drawn from swifts or the like 12, supported in any desired manner, through suitable cleaning, washing, and drying means

shown housed in a hood 14, whence they pass over a guide roller 16 into a bath 18 of molten zinc 20 covered by insulating material 22 such as expanded mica (known commercially as "Zonolite"). The zinc may heat a temperature of about 5 840° F. The wires are forced into the zinc by any suitable means such as a sinker 24 and may have excess zinc removed therefrom as they leave the bath, by suitable wipers 26.

As explained in my Patents Nos. 2,002,261, 10 2,002,262, and 2,002,263, some of the advantages of my invention are obtainable with other metals than zinc and copper. The invention described herein is capable of utilization with the various metals and plating-bath formulas described in 15 those patents; for most purposes, however, I prefer to galvanize on the wires a plating of zinc and then apply to the zinc-plated wires an electrolytically deposited coating of copper.

The wires remain in the zinc bath long enough 20 not only to receive their zinc coatings but also to be raised substantially to the temperature of the molten zinc, or at least near enough thereto to pass as described below into the copper cyanide or equivalent solution at the desired high tem- 25 perature.

Preferably, as the wires leave the zinc bath, the zinc coatings are set and solidified (without substantially lowering the temperature of the wires) by passing them over a quenching roller 30 28 having its bottom immersed in water in a trough 30.

In order to make the apparatus as compact as possible, I prefer to arrange the copper plating apparatus described below beside the above- 35 describe zinc-plating apparatus, leading the wires thereto around two right-angle bends formed by series of guide rollers (not specifically illustrated) arranged at 32 and 34.

The copper plating, or equivalent electrolytic 40 plating, apparatus illustrated is of novel form and arrangement designed to insure a continuous supply of fresh plating solution to the wires being plated. The apparatus may include a relatively long lower bath or tank 36, containing a 45 supply of an aqueous solution of copper cyanide containing, for example, about 30 to 35 grams of copper and 20 to 24 grams of cyanide per liter. I find that this solution operates best at a temperature of about 160° F. As explained below, 50 part of the necessary heat is derived from the hot wires 10.

The solution is continuously fed from the lower tank 36, by means such as one or more pumps 38 shown as driven by motors 40, to the centers 55

of novel shorter upper tanks 42, arranged end to end in a series above the solution in the tank 36. The solution in the tanks 42 flows both ways along the wires 10, and overflows back to the lower tank 36 through notches 44 in the ends of the tanks 42. The wires 10 are arranged in the notches 44.

The plating current passes (preferably at about 30 to 40 amperes per square foot of surface of the wires immersed in the plating solution) to the negative connection 48 to rolls 50 engaging and pressing down on the wires 10, supported by pairs of idler rollers 52 on opposite sides of the rolls 50, a series of rolls 50—52 so connected being arranged at each end of each of the upper tanks 42. The bottom of each roll 50 is slightly below the tops of the corresponding rolls 52, to insure good contact with the wires.

The positive current connection 54 is connected in the usual manner to copper plate electrodes 56 immersed in the solution in the upper tanks 42. These connections may have their resistances so balanced that substantially equal currents flow between the wires and the respective plates.

The hot wires, at approximately a temperature of around 650° to 700° F., i. e. greatly above the temperature of boiling water, thus pass directly into the plating solution in the first tank 42, the hot wires causing a very active reaction of the solution which clears off any traces of zinc oxide or other impurities immediately, and starts a very active deposition of the copper on the clean zinc surface, so that the copper is in such intimate contact with the zinc as readily to alloy therewith on standing, as explained in my above-identified patents, to form the desired brass surface.

The plated wires pass through suitable washing and drying means in a hood 60, and over suitable

devices 62 (illustrated diagrammatically as driven by motors 64) to wind them on swifts or the like 66.

The above-described process is also applicable to the electro-plating of zinc on a hot-galvanized wire from a bath of zinc cyanide, and to plating with other metals from an alkaline solution.

While one particular arrangement of the apparatus has been described in detail, it is not my intention to limit the scope of the invention by that description, or otherwise than by the appended claims.

I claim:

1. That method of plating a steel wire which comprises passing the wire through molten zinc to receive a zinc coating and at the same time be raised to a relatively high temperature, quenching the zinc coating without greatly lowering the temperature of the wire, passing the highly heated zinc-plated wire directly thereafter through a hot aqueous copper cyanide bath, and passing a current through the bath to the wire immersed therein, whereby the highly-heated wire as it enters the bath is cleared of impurities and is then plated with copper.

2. That method of plating a wire which comprises passing the wire through a molten metal to receive a metallic coating and at the same time be raised to a relatively high temperature, quenching the coating without greatly lowering the temperature of the wire, passing the highly heated plated wire directly thereafter through a hot aqueous metal-salt bath, and passing a current through the bath to the wire immersed therein, whereby the highly-heated wire as it enters the bath is cleared of impurities and is then plated with a second metal.

ELGIN CARLETON DOMM.